

1

3,160,484  
STABILIZING ADDITIVES FOR DISTILLATE  
FUELS

Joel R. Siegel, Elizabeth, N.J., assignor to Esso Research and Engineering Company, a corporation of Delaware  
No Drawing. Continuation of application Ser. No. 673,156, July 22, 1957. This application July 25, 1961, Ser. No. 126,531  
26 Claims. (Cl. 44—62)

The present invention relates to a new class of additives for use in petroleum distillate fuel products. More specifically, it relates to a new class of copolymers containing chlorine and to the use of such copolymers as additives for stabilizing petroleum distillate fuels. This application is a continuation of Serial No. 673,156, filed July 22, 1957.

It has long been recognized that heating oils, jet engine fuels and other middle distillate fuel products derived from petroleum often contain unstable compounds which tend to decompose and form sludge and sediment during storage. Fuels containing partially unsaturated stocks derived from thermal or catalytic cracking operations in quantities exceeding about 10 percent by volume are especially subject to such sludging and sedimentation. A number of different materials have been proposed heretofore for incorporation into such fuels in order to overcome their instability and avoid the plugging and fouling of fuel lines, filters and nozzles due to sediment and sludge. The most successful of these materials have been metallic compounds such as metal naphthenates, metal sulfonates, and metal salts of alkyl metal sulfides. Such metallic compounds, although effective for stabilizing fuels, are unsatisfactory because they leave a residue when burned. This residue leads to a gradual buildup of deposits in combination chambers and burner systems which materially decrease combustion efficiency. Various ashless compounds have been suggested in order to overcome these difficulties but have not been found wholly effective.

The present invention provides a new class of ashless additives containing chlorine which are effective in very small quantities for inhibiting the formation of sludge and sediment in petroleum distillate fuels boiling in the range between about 300° and about 900° F. Typical of such fuels are heating oils meeting the requirements for Grades 1 and 2 fuel oils as set forth in ASTM Specification D-396-48T, diesel fuels falling within Grades 1D, 2D and 4D of ASTM Specification D-975-51T, and jet engine fuels such as those covered by U.S. Military Specification MIL-F-5624C. The addition of as little as about 0.002 percent by weight of the additive materials of the invention significantly improves the stability of such fuels and extends the period for which they may be satisfactorily stored under adverse conditions.

The stabilizing additives of this invention are chlorine-containing copolymers containing ester groups derived from the reaction of epichlorohydrin with a carboxylic acid group. These copolymers may be prepared by copolymerizing with other polymerizable monomers or mixtures of such monomers the reaction product of epichlorohydrin with a polymerizable, unsaturated acid; i.e., dibasic acids such as maleic acid and half esters of dibasic acids such as lauryl hydrogen maleate. The chlorine-containing copolymers of the invention may also be prepared by the reaction of epichlorohydrin with polymers containing free carboxylic acid groups.

In a preferred embodiment of the invention, chlorine-containing copolymers are prepared by copolymerizing with polymerizable monomers mixed esters formed by reacting epichlorohydrin with an acid ester of an unsaturated conjugated dibasic acid.

2

The mixed esters which have been found useful in preparing copolymers for stabilizing petroleum distillate fuels in accordance with the invention are long chain saturated aliphatic alcohol-epichlorohydrin mixed esters of unsaturated conjugated dibasic acids. These esters, referred to hereinafter as alkyl-chloropropyleneoxy mixed esters are thought to have the general formula:



where R is an alkyl group containing from about 8 to about 24 carbon atoms; R' and R'' are constituents selected from the class consisting of hydrogen atoms and methyl groups, at least one such constituent being a hydrogen atom; and n may vary from one to three or more, depending upon the quantity of epichlorohydrin employed in preparing the esters.

The alkyl-chloropropyleneoxy mixed esters employed in preparing the copolymers of the invention may be readily obtained by first reacting an unsaturated conjugated dibasic acid with a long chain saturated aliphatic alcohol to form a half ester and then reacting this product with epichlorohydrin in the presence of an acidic (electron acceptor) catalyst to produce the mixed ester. The addition of epichlorohydrin to the half ester may also be catalyzed by basic groups, e.g.  $\text{CH}_3\text{O}^-$ ,  $\text{OH}^-$ . Suitable unsaturated conjugated dibasic acids for preparing the mixed esters in this manner include maleic acid, fumaric acid, citraconic acid, mesaconic acid, and mixtures of such acids. The butenedioic acids, i.e., maleic and fumaric acids and mixtures of the two, are preferred acids. It is preferable to employ the acids in the form of their anhydrides, in which case the half ester can be produced by merely heating one mole of the anhydride with one mole of the long chain saturated aliphatic alcohol at a temperature of about 70 to 120° C. for about thirty to about forty-five minutes. Other well-known methods for the production of half esters of dibasic acids may also be employed.

The long chain saturated aliphatic alcohols reacted with the dibasic acids or acid anhydrides to produce half esters may contain from about 8 to 24 carbon atoms per molecule, those containing from about 8 to about 18 carbon atoms being preferred. Straight chain primary alcohols such as dodecyl, cetyl, eicosyl and docosyl are preferred, but it is permissible to use branched alcohols such as 2-ethylhexanol-1 and  $\text{C}_8$  oxo-alcohols, secondary alcohols such as capryl alcohol and mixtures of straight and branched-chain alcohols if desired.

Commercially marketed mixtures of alcohols consisting essentially of saturated aliphatic alcohols having the requisite chain length may also be used. One such preferred mixture prepared by the hydrogenation of coconut oil is sold under the trade-name "Lorol" and is comprised of saturated aliphatic alcohols containing from 10 to 18 carbon atoms per molecule. This mixture consists chiefly of lauryl alcohol having 12 carbon atoms per molecule and has the following approximate composition:

| Number of carbon atoms: | Weight percent |
|-------------------------|----------------|
| $\text{C}_{10}$         | 4.0            |
| $\text{C}_{12}$         | 55.5           |
| $\text{C}_{14}$         | 22.5           |
| $\text{C}_{16}$         | 14.0           |
| $\text{C}_{18}$         | 4.0            |

Lorol is thus a commercial mixture of saturated aliphatic alcohols containing from 10 to 18 carbon atoms per molecule and having an average chain length of 12-14.

The  $\text{C}_8$  oxo-alcohol effective for use in preparing the

additives of the invention are normally obtained by the oxonation and hydrogenation of a C<sub>7</sub> copolymer of propylene and butene. The copolymer itself is in reality a mixture of isomers and the resultant oxo-alcohol may have the following general analysis:

STRUCTURE OF C<sub>8</sub> OXO-ALCOHOL PREPARED FROM C<sub>8</sub>-C<sub>4</sub> COPOLYMER HEPTENES

| Constituent                  | Percent |
|------------------------------|---------|
| <chem>CC(C)C(O)CC(C)C</chem> | 29      |
| <chem>CC(C)C(O)CC(C)C</chem> | 25      |
| <chem>CC(C)C(O)CC(C)C</chem> | 17      |
| <chem>CC(C)C(O)CC(C)C</chem> | 16      |
| <chem>CC(C)C(O)CC(C)C</chem> | 2.3     |
| <chem>CC(C)C(O)CC(C)C</chem> | 1.4     |
| 2-alkyl alkanols             | 4.3     |
| Others                       | 5.0     |
|                              | 100.0   |

Higher molecular weight oxo-alcohols may also be used in preparing the additives of the invention. These higher molecular weight alcohols are believed to have compositions generally analogous to that specified above, chain lengths and degree of branching depending upon the type of olefins used in preparing the copolymers. The process used for the manufacture of oxo-alcohols is now well-known in the art and need not be further described.

The half esters prepared by reacting the dibasic acid and alcohol are in turn reacted with epichlorohydrin in the presence of from about 0.05 to 5.0 percent by weight of an acidic (electron acceptor) catalyst such as boron trifluoride, boron trifluoride etherate, aluminum trichloride, aluminum tribromide or the like or a basic catalyst such as NaOCH<sub>3</sub> or NaOH. The reaction is carried out by slowly adding the epichlorohydrin to the half ester mixed with catalyst over approximately a one to two hour period. The temperature at which the addition is carried out may range between about 100° C. and 180° C. The reactants are held at this temperature from about 4 hours to about 24 hours or longer. Depending upon the number of chlorine atoms desired per molecule of mixed ester, the ester:epichlorohydrin ratio may range between about 1:1 to about 1:4. Under these conditions the addition of the epichlorohydrin molecule to the half ester takes place through the epoxy group and the chlorine atom of the epichlorohydrin is unaffected.

It is preferred that the half ester and the epichlorohydrin be reacted in substantially equimolar quantities so that the mixed ester contains a single chloropropyleneoxy group. It has been found that the stabilizing properties of the mixed ester are not greatly improved by the presence of more than one chloropropyleneoxy group per molecule. The reaction may be carried out in a suitable solvent such as benzene, toluene, xylene or the like if desired, although ordinarily the use of such a solvent is not necessary. The mixed ester thus produced may be washed with a dilute solution of sodium hydroxide if the

catalyst used was acidic or dilute acid if the catalyst was basic and then water washed.

The mixed esters prepared as described above are copolymerized with a polymerizable organic monomer containing a vinyl group in order to produce stabilizing additives for incorporation in petroleum distillate fuels. Suitable monomers containing vinyl groups include hydrocarbons such as styrene, isobutylene, and butadiene; esters such as allyl acetate, vinyl propionate and methyl methacrylate; ethers such as allyl ethyl ether and divinyl ether; nitriles such as acrylonitrile and vinylacetonitrile. Mixtures of such monomers containing vinyl groups with other copolymerizable materials, long chain alcohol esters of unsaturated conjugated dibasic acids such as lauryl maleate and tallow fumarate for example, may also be used. Vinyl esters of short chain fatty acids, particularly vinyl acetate, and mixtures of such esters with fumarate or maleate esters of long chain aliphatic alcohols containing from about 8 to 20 carbon atoms per molecule are preferred monomers for the preparation of copolymers with the mixed esters.

The copolymerization of the mixed ester with the organic monomer may be carried out in a solution of benzene or other suitable organic solvent at a temperature in the range of from about 60° to about 250° F. and may be promoted by gamma radiation or by the use of a peroxide type catalyst such as benzoyl peroxide, a hydroperoxide or an azo catalyst such as alpha-alpha' azo-bisisobutyronitrile. The mole ratio of mixed ester to other organic monomers in the polymerization mixture may be varied from about 2:1 to about 1:20. The polymerization may be carried out in a suitable solvent in order to control reaction velocity and molecular weight. Oxygen generally will be excluded during the polymerization by the use of a blanket of an inert gas such as nitrogen or carbon dioxide. The polymerization time may vary from about 1 to 36 hours.

Polymerization of the mixed ester and the organic monomer proceeds between the unsaturated double bonds in the acid portion of the ester and in the monomer. The copolymer may have molecular weights of from about 3000 to about 100,000 or higher. The molecular weight can be determined by measuring the viscosity of diisobutylene solutions containing 5 mg. of the copolymer per cc. and applying the Staudinger equation. Molecular weights of from about 6,000 to about 20,000 are particularly preferred. Upon completion of the polymerization reaction, the copolymer may be freed of solvent and employed for the stabilizing of distillate fuels.

The copolymer may be incorporated into petroleum distillate fuels in concentrations of from about 0.002 to about 2 percent by weight in order to stabilize such fuels. At these concentrations the copolymers of the invention are oil-soluble and may therefore be added directly to the fuel. A solvent such as kerosene or the like may be used to facilitate handling if desired, however.

Concentrations of from about 0.005 to about 0.1 percent by weight are normally adequate and are preferred.

The following examples will serve to illustrate the stabilizing action of the additive of the invention.

EXAMPLE 1

Isooctyl chloropropyleneoxy maleate was prepared by reacting epichlorohydrin and isoctyl hydrogen maleate, an acid-ester of isoctyl alcohol and maleic acid, in the presence of 0.05 wt. percent of a sodium methylate catalyst. One mole of the epichlorohydrin was added to one mole of the acid ester in a stirred reaction vessel containing the catalyst over a period of about one hour. The addition temperature was 165° C. The reaction mixture was then maintained at this temperature for a period of 7 hours. At the end of this time it was found that substantially all the reactants had been converted to the mixed ester. A chlorine analysis of the product showed that the mixed ester contained essentially one epichlorohydrin

group per molecule of the ester. The Total Acid Number and the Saponification Number of the product were as follows:

|                  | Calc. | Found |
|------------------|-------|-------|
| TAN, mg. KOH/gm. | 0     | 4.9   |
| SAP, mg. KOH/gm. | 525   | 433   |

## EXAMPLE 2

Isooctyl chloropropyleneoxy maleate was prepared by the method of Example 1 except that the catalyst used was 0.05 wt. percent of sodium hydroxide. The properties of the mixed ester product were essentially the same as those of the product of the preceding example. The 15 mixed ester had the following Total Acid Number and Saponification Number:

|                  | Calc. | Found |
|------------------|-------|-------|
| TAN, mg. KOH/gm. | 0     | 3.1   |
| SAP, mg. KOH/gm. | 525   | 437   |

## EXAMPLE 3

Epichlorohydrin and isoctyl hydrogen maleate, an acid-ester of isoctyl alcohol and maleic acid, were reacted to form a mixed ester by adding to one mole of the half ester in the presence of 0.5% by wt. of  $BF_3$  etherate one mole of epichlorohydrin over a period of about one hour. This was carried out with stirring at a temperature of about 150° C. This temperature was held for about 17 hours. Analysis of the mixed ester thus produced showed that the ester contained approximately one molecule of epichlorohydrin per molecule of ester. The Saponification Number and the Total Acid Number of the mixed ester, expressed as milligrams of KOH per gram of sample, were 417.8 and 9.1 respectively, as compared to calculated values of 525 and 0 respectively. A copolymer of this ester (.125 mole) with vinyl acetate (1 mole) and tallow fumarate (.875 mole), fumaric acid esterified with a mixture of saturated aliphatic alcohols containing from 16 to 18 carbon atoms per molecule, was prepared by heating the reactants in an equal weight of benzene for about 3 hours at 80°-90° C. in the presence of 1 weight percent of benzoyl peroxide.

## EXAMPLE 4

Employing the reactants of Example 3, a polymer containing 0.25 mole of isoctyl chloropropyleneoxy maleate and 0.75 mole of tallow fumarate per mole of vinyl acetate was prepared. The reaction conditions and catalyst were the same as those of Example 3 except that the mixture was heated for 1.5 hours.

## EXAMPLE 5

Equimolar quantities of epichlorohydrin and tallow hydrogen maleate were reacted to form a mixed ester in accordance with the method of Example 3. A copolymer of this ester with vinyl acetate and tallow fumarate containing 0.125 mole of the mixed ester and 0.875 mole of tallow fumarate per mole of vinyl acetate was then prepared.

## EXAMPLE 6

The reactants employed in Example 5 were copolymerized to give a copolymer containing 0.25 mole of a mixed ester and 0.75 mole of tallow fumarate per mole of vinyl acetate.

## EXAMPLE 7

Lorol hydrogen maleate, an acid ester of maleic acid and a mixture of saturated  $C_{12}$  to  $C_{18}$  aliphatic alcohols derived from the hydrogenation of coconut oil, was reacted with epichlorohydrin in equimolar quantities by heating the reactants after slow addition of the epichlorohydrin to the half ester in xylene solution in the presence of 1 percent by weight of boron trifluoride etherate catalyst. The re-

action was carried out at a temperature of 155° C. and was continued for 17 hours. The resulting mixed ester was washed with 5 percent sodium hydroxide in water and then dried. The Total Acid Number of the mixed ester, expressed as milligrams of KOH per gram of the ester, was 4.5, against a calculated value of zero. The mixed ester contained 5.5% chlorine against a calculated value of 6.7% by weight. The product from this reaction was mixed with vinyl acetate in a molar ratio of 1.4 moles of vinyl acetate per mole of ester in 50 percent by weight of benzene. One percent by weight of benzoyl peroxide was added to the solution as a catalyst and the reaction mixture was then exposed to 6 megaroentgens of gamma radiation at 110° F. to effect copolymerization.

## EXAMPLE 8

The copolymers prepared in Examples 3, 4, 5, 6 and 7 were incorporated at a concentration of 0.01% by weight of the 50% benzene solution into samples of a heating oil comprising a blend of about 50 percent virgin distillate and about 50 percent cracked stock. Typical properties of such a heating oil are as follows:

|                     |     |
|---------------------|-----|
| Gravity, API        | 32  |
| Color, Tag-Robinson | 13  |
| Flash, ° F.         | 150 |
| Sulfur, percent     | 0.8 |
| Aniline point, ° F. | 137 |
| Distillation, ° F.: |     |
| IBP                 | 330 |
| 10%                 | 420 |
| 50%                 | 500 |
| 90%                 | 585 |
| FBP                 | 645 |

These samples and a sample of the base oil were subjected to an Accelerated Storage Stability Test which comprised heating the samples for a period of 16 hours at a temperature of 210° F. At the end of the 16 hour period the samples were filtered through a medium porosity sintered glass filter and the amount of sediment formed was determined.

TABLE I  
Accelerated Storage Stability Tests

[Additive conc.=.01% of a 50% solution in benzene]

|                                      |                          |
|--------------------------------------|--------------------------|
| Additive:                            | Sediment, mg./600 g. oil |
| None                                 | 12.7                     |
| Product of Example 3                 | 1.2                      |
| Product of Example 4                 | 1.4                      |
| Product of Example 5                 | 1.0                      |
| Product of Example 6                 | 0.8                      |
| Product of Example 7                 | 1.6                      |
| Reproducibility of test, $\pm 1$ mg. |                          |

As shown by these data, the additives of the invention substantially reduced sediment formation in the oil.

## EXAMPLE 9

The additives of the invention are effective in jet fuels as well as in middle distillate heating oils. To demonstrate this, the products of Examples 3 and 4 were incorporated into samples of a jet fuel covered by U.S. Military Specification MIL-F-5624C which boiled between 300 and 550° F. These samples were subjected to a CFR Fuel Coker Test. The tests were carried out by passing the samples through hot preheater tubes which brought the fuel temperature to 400° F. The heated fuel was then passed through a sintered metal micronic filter heated to a temperature of 500° F. The pressure drop across the filter and the deposit formed on the preheater tubes were measured for each sample and compared with the values obtained with the uninhibited fuel. Data from this test are shown in Table II.

TABLE II  
Fuel Coker Stability Tests

| Additive                                 | Coker Merit Rating <sup>1</sup> | Preheater Tube Deposits <sup>2</sup> |
|------------------------------------------|---------------------------------|--------------------------------------|
| None                                     | 100                             | 50/8                                 |
| Prod. of Ex. 3, 0.01% Active ingredient  | 750                             | 75/5                                 |
| Prod. of Ex. 4, 0.005% Active ingredient | 710                             | 75/5                                 |
| Prod. of Ex. 4, 0.01% Active ingredient  | 740                             | 35/7                                 |

<sup>1</sup> A rating of 500 or above is considered good.

<sup>2</sup> First number is percent tube covered, second is color of deposit:  
0=clear; 2=very light tan; 4=tan; 6=brown; 8=dark brown; 10=black.

EXAMPLE 10

To demonstrate the stabilizing action of the additives of the invention still further, fuel oil samples containing the products prepared in the previous examples and a commercial additive of the ashless type were subjected to an Accelerated Filter Plugging test by aging the samples for a period of 16 hours to a maximum temperature of 230° F. and then filtering them. The pressure drop across the filter pads, the weights of sediment recovered and the color of the sediment on the pads were noted and compared. Table IV shows the results obtained in this test.

TABLE III  
Accelerated Filter Plugging Test

| Additive                      | Demerit Rating |        |          |         |
|-------------------------------|----------------|--------|----------|---------|
|                               | ΔP             | Visual | Sediment | Overall |
| None                          | 4              | 5      | 3        | 4.0     |
| Product of Example 3 (0.005%) | 0              | 0      | 1        | 0.3     |
| Product of Example 3 (0.01%)  | 0              | 2      | 0        | 0.7     |
| Product of Example 4 (0.007%) | 0              | 1      | 0        | 0.3     |
| Product of Example 4 (0.01%)  | 0              | 2      | 0        | 0.7     |
| Product of Example 5 (0.01%)  | 0              | 1      | 0        | 0.3     |
| Product of Example 6 (0.01%)  | 0              | 1      | 0        | 0.3     |
| Product of Example 7 (0.01%)  | 0              | 1      | 1        | 0.7     |
| Ashless Commercial Additive   | 0              | 2      | 0        | 0.7     |

The test employed is described in detail in "New Fast Test Method for Distillate Storage Stability," by W. A. Konrad, N. L. Shipley and T. S. Tutwiler, which is found on page 145 of Petroleum Processing, September 1956.

The lower the value of the overall demerit rating in this test, the better the stability properties of the oil. Again it can be seen that the additives of the invention produce a marked improvement in the stability of distillate fuels and in some respects are superior to commercial additives.

It will be understood that the additives of the invention may be incorporated into petroleum distillate fuels in conjunction with other additives designed to correct other fuel deficiencies. The additives may also be used in the form of amine or other derivatives rather than as straight copolymers.

What is claimed is:

1. A copolymer of a long chain saturated aliphatic alcohol-chloropropyleneoxy mixed ester of an unsaturated conjugated dibasic acid, said acid having from 4 to 5 carbon atoms per molecule and a polymerizable organic monomer selected from the group consisting of (a) a vinyl ester of a short chain fatty acid and (b) a mixture of a vinyl ester of a short chain fatty acid and a long chain saturated aliphatic alcohol ester of a conjugated unsaturated dibasic acid, said acid containing from 4 to 5 carbon atoms per molecule, and wherein the mole ratio of said mixed ester to said monomer is between 2:1 and 1:20, and said copolymer has a molecular weight of from 3,000 to about 100,000.

2. A copolymer as defined in claim 1 wherein the said vinyl ester of a short chain fatty acid is vinyl acetate.

3. A copolymer as defined in claim 1 wherein said unsaturated conjugated dibasic acid is a butenedioic acid.

4. A copolymer as defined in claim 1 wherein said long chain saturated aliphatic alcohol is a straight chain primary alcohol containing from 8 to 24 carbon atoms per molecule.

5. A copolymer as defined in claim 1 wherein the said copolymer has a molecular weight of between 6,000 and about 20,000.

6. A copolymer as defined in claim 1 wherein the mixed ester to chloropropyleneoxy ratio is between 1:1 to about 1:4.

7. An oil soluble copolymer of an alkyl C<sub>8</sub> to C<sub>24</sub> chloropropyleneoxy mixed ester of a butenedioic acid having a mixed ester to chloropropyleneoxy ratio of between 1:1 and 1:4 and a monomer selected from the group consisting of (a) vinyl acetate and (b) a mixture of vinyl acetate and a C<sub>8</sub> to C<sub>20</sub> saturated aliphatic ester of a butenedioic acid, said copolymer having a mole ratio of mixed ester to monomer of between 2:1 and 1:20 and a molecular weight between 6,000 and about 20,000.

8. An oil soluble copolymer of an alkyl C<sub>8</sub> to C<sub>20</sub> chloropropyleneoxy maleate and a vinyl acetate, said copolymer having a mole ratio of maleate to acetate of between 2:1 and 1:20 and having a molecular weight of 6,000 to about 20,000.

9. An oil soluble copolymer of an alkyl C<sub>8</sub> to C<sub>24</sub> chloropropyleneoxy maleate and a monomeric mixture of vinyl acetate and alkyl fumarate, said copolymer having a mole ratio of maleate to monomer mixture of between 2:1 and 1:20 and a molecular weight between 6,000 and about 20,000.

10. A copolymer of a long chain saturated aliphatic alcohol-chloropropyleneoxy mixed ester of an unsaturated conjugated dibasic acid, said acid having from 4 to 5 carbon atoms per molecule and styrene and wherein the mole ratio of said mixed ester to styrene is between 2:1 and 1:20 and said copolymer has a molecular weight of between 3,000 and 100,000.

11. A copolymer of a long chain saturated aliphatic alcohol-chloropropyleneoxy mixed ester of an unsaturated conjugated dibasic acid, said acid having from 4 to 5 carbon atoms per molecule and methyl methacrylate and wherein the mole ratio of said mixed ester to methyl methacrylate is between 2:1 and 1:20 and said copolymer has a molecular weight of between 3,000 and 100,000.

12. A petroleum distillate fuel boiling in the range between about 300° F. and about 900° F. having incorporated therein a stabilizing amount of a copolymer of a long chain saturated aliphatic alcohol-chloropropyleneoxy mixed ester of an unsaturated conjugated dibasic acid, said acid having from 4 to 5 carbon atoms per molecule and a polymerizable organic monomer selected from the group consisting of (a) a vinyl ester of a short chain fatty acid and (b) a mixture of a vinyl ester of a short chain fatty acid and a long chain saturated aliphatic alcohol ester of a conjugated unsaturated dibasic acid, said acid containing from 4 to 5 carbon atoms per molecule, and wherein the mole ratio of said mixed ester to said monomer is between 2:1 and 1:20, and said copolymer has a molecular weight of from 3,000 to about 100,000.

13. A fuel composition as defined by claim 12 wherein in the concentration of said copolymer is from about 0.002 to 2 percent by weight.

14. A fuel composition as defined by claim 12 wherein in said mixed ester is Lorol-chloropropyleneoxy maleate.

15. A fuel composition as defined by claim 12 wherein in said vinyl ester comprises vinyl acetate.

16. A fuel composition as defined by claim 12 wherein in said mixed ester is isoctyl chloropropyleneoxy maleate.

17. A fuel composition as defined by claim 12 wherein in said mixed ester is tallow-chloropropyleneoxy maleate.

18. A fuel composition as defined in claim 12 wherein in said unsaturated conjugated dibasic acid is a butenedioic acid.

19. A fuel composition as defined in claim 12 wherein in said long chain saturated aliphatic alcohol is a straight

chain primary alcohol containing from 8 to 24 carbon atoms per molecule.

20. A fuel composition as defined in claim 12 wherein the said copolymer has a molecular weight of between 6,000 and about 20,000.

21. A fuel composition as defined in claim 12 wherein the mixed ester to chloropropyleneoxy ratio is between 1:1 to about 1:4.

22. A fuel composition as defined in claim 12 wherein said distillate fuel is a jet fuel boiling in the range between about 300° F. and about 550° F.

23. A petroleum distillate fuel boiling in the range between about 300° F. and about 900° F. having incorporated therein from about 0.002 to about 2.0% by weight of an oil soluble copolymer of an alkyl C<sub>8</sub> to C<sub>24</sub> chloropropyleneoxy mixed ester of a butenedioic acid having a mixed ester to chloropropyleneoxy ratio of between 1:1 and 1:4 and a monomer selected from the group consisting of (a) vinyl acetate and (b) a mixture of vinyl acetate and a C<sub>8</sub> to C<sub>20</sub> saturated aliphatic ester of a butenedioic acid, said copolymer having a mole ratio of mixed ester to monomer of between 2:1 and 1:20 and a molecular weight between 6,000 and about 20,000.

24. A petroleum distillate fuel boiling in the range between about 300° F. and about 900° F. to which has been added from about 0.005 to about 0.1 percent by weight of a copolymer of a mixed ester of tallow-chloropropyleneoxy maleate with an organic monomer mixture of 1 mole of vinyl acetate and 0.75 to 0.875 mole of tallow fumarate and wherein the mole ratio of ester to monomer is between 2:1 and 1:20, said copolymer having a molecular weight of from about 6,000 to about 20,000 Staudinger.

25. A petroleum distillate fuel boiling in the range between about 300° F. and about 900° F. to which has

5  
10

been added from about 0.005 to about 0.1 percent by weight of a copolymer of a mixed ester of isoctyl chloropropyleneoxy maleate, with an organic monomer mixture of 1 mole of vinyl acetate and 0.75 to 0.875 mole of tallow fumarate and wherein the mole ratio of ester to monomer is between 2:1 and 1:20, said copolymer having a molecular weight of from about 6,000 to about 20,000 Staudinger.

26. A petroleum distillate fuel boiling in the range between about 300° F. and about 900° F. to which has been added from about 0.005 to about 0.1% by weight of a copolymer of a mixed ester of Lorol-chloropropyleneoxy maleate with an organic monomer of vinyl acetate wherein the mole ratio of ester to monomer is between 2:1 and 1:20, said copolymer having a molecular weight of from 6,000 to 20,000 Staudinger.

#### References Cited in the file of this patent

#### UNITED STATES PATENTS

|           |                  |               |
|-----------|------------------|---------------|
| 2,402,863 | Zuidema et al.   | June 25, 1946 |
| 2,448,531 | Kenyon           | Sept. 7, 1948 |
| 2,524,432 | Dorough          | Oct. 3, 1950  |
| 2,539,438 | Kropa et al.     | Jan. 30, 1951 |
| 2,607,761 | Seymour          | Aug. 19, 1952 |
| 2,615,845 | Lippincott       | Oct. 28, 1952 |
| 2,626,945 | Carlin           | Jan. 27, 1953 |
| 2,642,414 | Bauer et al.     | June 16, 1953 |
| 2,800,401 | Lusebrink et al. | July 23, 1957 |

#### OTHER REFERENCES

Industrial and Engineering Chemistry, vol. 41, No. 17, July 1949, "Copolymers of Vinyl Compounds and Maleic Anhydride," by Seymour et al., pages 1509-1513.